# EUROPEAN PATENT APPLICATION

(11) **EP 1 319 484 A1**
(43) Date of publication of application: **18.06.2003**
(21) Application number: 02027041.9
(22) Date of filing: 03.12.2002
(51) Int. Cl.: B27N 7/00

(54) **Method and plant for facing panel surfaces with melaminic of phenolic paper sheets**

(30) Priority: 11.12.2001 IT MI20012603
(71) Applicant: PAGNONI IMPIANTI S.p.A., 20124 Milano (IT)
(72) Inventor: Pagnoni, Giorgio, 20052 Monza (MI) (IT)
(74) Representative: Faraggiana, Vittorio, Dr. Ing.

(57) **Abstract**

A plant for quick facing wood-based panel surfaces with melaminic or phenolic paper sheets comprises a press (11), and a sequential contact-cooling unit (12). The press is operated for hot-pressing of a pack formed of a wooden panel and one or more paper sheets. The cooling unit (12) comprises superposed faced plates (17, 18) that are cooled to a preset temperature and can be closed to come into contact with the opposite faces of the pack after the latter comes out of the hot press. The cooling unit further comprises suction means (20) for the fumes given off from the pack disposed between the cooled plates. In accordance with the method, the press temperature is between 150 and 210°C and the temperature of the cooling plates is between 20 and 60°C, whereas the pressing pressure is in the range of 20 to 40 kg/cm². The cooled plates are closed onto the pack at a pressure between 1 and 2 kg/cm².

## Description

The present invention relates to a method and a plant for facing wood-based panel surfaces (chipboards, MDF, multilayered sheets) with melaminic or phenolic paper sheets.

The plants for facing panel surfaces with melaminic or phenolic paper sheets generally consist of hot-plate presses between which the paper/panel/paper sandwich is tightened and simultaneously submitted to the action exerted by pressure and temperature, so as to fluidise the resins (of the thermosetting type) and polymerise them on reaching of a given temperature (on the order of 150-180°C).

These presses are interlocked upstream and downstream with automatic devices for press loading and unloading. After pressing, the panels, still hot on their surfaces, are submitted to some finishing operations (trimming of the edges, possible cutting operations, brushing, etc.) and finally stacked up. If they are stacked up when their surface temperature is still high (in the order of 100°C), the subsequent cooling may happen to take place in an uneven manner, both from one panel to another and in different regions of the same panels. For example, cooling will be different between panels on top of the stack and panels in the middle and, as regards the last-mentioned case, it will be different on a panel periphery than in the central portion thereof.

Cooling unevennesses create stresses inside the panel that, on subsequent unpiling, cause deformation of the panel itself.

In the known art, the problem is usually solved by introducing cooling devices (of the so-called book-shaped or star-shaped type, depending on their construction) in the unloading lines before the piling-up operation, which cooling devices keep the panels exposed in the open air for 10-30 minutes before stacking them up. These cooling devices can also contemplate an exposure to a forced air stream to improve yield, but in this case there is the risk that the air stream may preferably only impinge on some regions of the panels thereby just causing those deformations that are wished to be avoided.

The cooling problem was still more felt since when in the facing plants production of the so-called floor panels was introduced, i.e. of panels adapted to form manufactured articles acting as substitutes for parquet.

Parquet is usually made up of strips of solid and valuable wood which is therefore very expensive. The "artificial or false parquet" is obtained from high-density MDF or chipboard panels surface-faced with paper sheets reproducing the pattern of the true parquet strips. In order to give the surface of the faced panels the necessary hardness and resistance to abrasion however, not only one paper sheet but a pack of 2-3 paper sheets are superposed on the panel, the uppermost paper sheet being transparent (to show the sheet under it carrying the wood pattern) and charged with particular and very strong resins.

These resins ask for longer baking times and therefore the panels during pressing absorb a greater heat amount which penetrates more deeply into the panel thickness and dispersion of which will be subsequently more difficult.

In addition, floor panels, as they are relatively thin (6-8 mm), are more subjected to deformation and their surfaces are faced with different types of paper sheets on the two faces (since the lower face is never in sight) and therefore, surface stresses are asymmetric. These panels, due to their final use, must not be absolutely subjected to deformation over time, i.e. after installation of same with the final user, because this fact would cause a very serious damage to the producer's image.

Due to the above discussed matter, manufacturers of floor panels are very careful about the problem of deformation and therefore about panel cooling before piling up, trying to do their best to make exposure to the cooling air in the above mentioned cooling devices as uniform as possible.

Although hot-cold multipress systems have been proposed in the case, of different nature, of high-pressure pressing operations for layered rolled sections, for several reasons the operating parameters of these systems were not found suitable for pressing faced panels.

It is an aim of the present invention to obviate the above mentioned drawbacks, by providing a method and a plant for production of faced panels enabling achievement of excellent results while avoiding the problem of deformation in spite of a quick production cycle.

In view of the above aim in accordance with the invention, a method has been conceived for quick facing surfaces of wood-based panels with melaminic or phenolic paper sheets, comprising the steps of pressing a pack formed of one wood-based panel and one or more of said paper sheets to a first pressure by a press heated to a first preset temperature and then causing passage of the pack through a contact-cooling unit comprising faced plates that are cooled to a second preset temperature and can be closed towards each other to come into contact with the opposite faces of the pack after the latter comes out of the hot press, the first temperature being included between 150 and 210°C, the second temperature being included between 20 and 60°C, and the first pressure being in the range of 20 to 40 kg/cm².

Still in accordance with the invention, a plant has been conceived for quick facing surfaces of wood-based panels with melaminic or phenolic resins, comprising a press heated to a first preset temperature for hot-pressing, and a sequential contact-cooling unit, the press being operated for hot pressing to a first pressure of a pack formed of a wood-based panel and one or more of said paper sheets, the cooling unit comprising superposed faced plates that are cooled to a second preset temperature and can be closed towards each other to come into contact with the opposite faces of the pack after the pack comes out of the hot press, the cooling unit comprising suction means for the fumes given off from the pack disposed between the cooled plates, at least before closure of said cooled plates.

For better explaining the innovative principles of the present invention and the advantages it offers over the known art, a possible embodiment applying said principles will be described hereinafter, by way of example, with the aid of the accompanying drawings. In the drawings:
- Fig. 1 is a diagrammatic elevation side view of a plant in accordance with the invention;
- Fig. 2 is a cross-sectional view taken along line II-II in Fig. 1;
- Fig. 3 is an enlarged diagrammatic view of a detail of the plant in Fig. 1.

With reference to the drawings, diagrammatically shown in Fig. 1 is a plant (generally identified by 10) for quick facing surfaces of wood-based panels with melaminic or phenolic paper sheets. The plant comprises a heated press 10 (essentially of known type and therefore not further described or shown) and a contact-cooling unit 12 sequentially disposed after the press. Possibly, placed between the press and cooling unit is a conveyor 13 for transfer of packs 14 formed of the wood panels 15 and the associated facing sheets (disposed on one or both faces of the panel).

The press is heated to a first preset temperature for hot pressing to a first pressure of a pack placed thereon.

The cooling unit 12 comprises superposed faced plates 17, 18 that are cooled to a second preset temperature by an appropriate fluid circulating therein. The plates can be closed towards each other by actuators 19 for coming into contact with the opposite faces of the pack after the pack comes out of the hot press.

It was found that for obtaining a stable product devoid of deformations over time the press temperature must be included between 150 and 210°C and the pressing pressure must be included between 20 and 40 kg/cm². In addition, the temperature in the cooling unit must be included between 20 and 60°C. It was found advantageous for the cooling plates to be pushed onto the pack surfaces to a pressure in the range of 1 to 2 kg/cm².

At each pressing cycle, the heated press is advantageously maintained closed on the pack for a period of time of 10 to 40 seconds, whereas the cooled plates are maintained closed on the pack for a period of time of 5 to 35 seconds.

The surface temperature of the panels immediately after they come out of the press is therefore approximately 100-150°C and the temperature conveniently reached on the panel surface before piling up of said panels is less than 50-70°C.

As shown in Fig. 2 and in more detail in Fig. 3, the cooling unit 12 comprises means 20 for suction of the fumes emitted from the pack disposed between the cooled plates. This suction means is operated at least before closure of the cooled plates, to remove possible fumes before they may condense due to cooling of the pack. It was found in fact that condensate causes deformation and unacceptable spots on the finished product.

Advantageously, the suction means is disposed around at least part of the periphery of the upper cooled plate and comprises a pipeline 21 disposed along the edge of the upper plate and provided with a plurality of holes 22 for forced suction.

It was also found advantageous for the suction means to be maintained in operation after closure of the cooled plates too, so as to capture the residual fumes that may be emitted from the edge of the pack submitted to cooling.

At this point it is apparent that the intended purposes have been achieved by providing a system enabling quick achievement of a temperature suitable for piling up the faced panels, without the risk of producing deformations or inner stresses that may give rise to subsequent deformations both in the short-term and in the long-term.

Obviously, the above description of an embodiment applying the innovative principles of the present invention is given by way of example only and therefore must not be considered as a limitation of the patent rights herein claimed. For example, the sizes, proportions and arrangement of the plant parts can vary depending on practical specific requirements.

## Claims

1. A method for quick facing surfaces of wood-based panels with melaminic or phenolic paper sheets, comprising the steps of pressing a pack formed of one wood-based panel and one or more of said paper sheets to a first pressure by a press heated to a first preset temperature and then causing passage of the pack through a contact-cooling unit comprising faced plates that are cooled to a second preset temperature and can be closed towards each other to come into contact with the opposite faces of the pack after the latter comes out of the hot press, the first temperature being included between 150 and 210°C, the second temperature being included between 20 and 60°C, and the first pressure being in the range of 20 to 40 kg/cm².

2. A method as claimed in claim 1, wherein the cooled plates are closed onto the pack to a pressure between 1 and 2 kg/cm².

3. A method as claimed in claim 1, wherein during each pressing the heated press is maintained closed on the pack for a time included between 10 and 40 seconds.

4. A method as claimed in claim 1, wherein the cooled plates are maintained closed on the pack for a time included between 5 and 35 seconds.

5. A method as claimed in claim 1, wherein the surface temperature of the panels after the panels come out of the press and before cooling in the cooling unit is approximately 100-150°C.

6. A method as claimed in claim 1, wherein the temperature reached on the panel surface before a subsequent piling-up operation is less than 50-70°C.

7. A method as claimed in claim 1, wherein at least before closure of the cooled plates, suction of the fumes given off from the pack disposed between said plates is carried out.

8. A method as claimed in claim 7, wherein suction also goes on after closure of the cooled plates to capture the residual fumes emitted from the edge of the pack submitted to cooling between said plates.

9. A plant for quick facing surfaces of wood-based panels with melaminic or phenolic resins, comprising a press heated to a first preset temperature for hot-pressing, and a sequential contact-cooling unit, the press being operated for hot pressing to a first pressure of a pack formed of a wood-based panel and one or more of said paper sheets, the cooling unit comprising superposed faced plates that are cooled to a second preset temperature and can be closed towards each other to come into contact with the opposite faces of the pack after the latter comes out of the hot press, the cooling unit comprising suction means for the fumes given off from the pack disposed between the cooled plates, at least before closure of said cooled plates.

10. A plant as claimed in claim 9, **characterised in that** the first temperature is included between 150 and 210°C, the second temperature is included between 20 and 60°C, the first pressure is in the range of 20 to 40 kg/cm², and the cooled plates are closed onto the pack at a pressure of 1 to 2 kg/cm².

11. A plant as claimed in claim 7, **characterised in that** said suction means is disposed around at least part of the periphery of the upper cooled plate.

12. A plant as claimed in claim 11, **characterised in that** the suction means comprises a pipeline with a plurality of holes for forced suction around at least part of the periphery of the upper plate.

13. A plant as claimed in claim 9, **characterised in that** the suction means is maintained in operation after closure of the cooled plates too, for capturing the residual fumes given off from the edge of the pack submitted to cooling between said plates.
